

Aug. 2, 1966

R. W. KIRKPATRICK

3,263,287

METHOD OF PREPARING MOLDS

Filed Nov. 3, 1964



FIG. 2



INVENTOR  
RICHARD W. KIRKPATRICK

By Donald G. Dalton  
Attorney

1

3,263,287

**METHOD OF PREPARING MOLDS**

Richard W. Kirkpatrick, North Canton, Ohio, assignor to  
United States Steel Corporation, a corporation of  
Delaware

Filed Nov. 3, 1964, Ser. No. 408,578  
4 Claims. (Cl. 22—192)

This invention relates to an improved method of preparing molds used in the manufacture of cast iron rolls.

A conventional mold used in forming a cast iron roll includes a cast iron "chill" in which the roll body is formed, and a sand "drag" and "cope" in which necks are formed at opposite ends of the body. The mold is placed in an upright position with the drag at the bottom and the cope at the top, and molten iron poured through a gate in the drag. The iron swirls as it rises through the mold to fill the chill and cope. Contact with the chill rapidly cools the outside of the body to produce a hard case. The remainder of the roll casting cools more slowly to provide toughness.

The chill must be preheated above ambient temperature before the molten iron is introduced to prevent its cracking because of the extreme temperature difference. Commonly the chill is preheated to about 600° to 800° F., and the molten iron poured at about 2800° F. It is essential that the chill have a rust-free surface, since any rust spots leave defects in the roll casting. The cope and drag are formed with sand which contains about 8 to 8.5 percent moisture. Before the molten iron is poured, the sand must be dried almost completely and it must be free of defects such as blow holes caused by overly rapid vaporization of moisture during the drying operation. Thus it is necessary to heat both the metal and sand parts of the mold under controlled conditions which do not rust the metal, and which fully dry the sand without producing defects. Previous practice has been to heat the mold parts in recirculating-type heaters in which products of combustion do not contact the parts directly. Direct-fired heaters are more efficient, but their use produced rust spots on the chills and defects in the sand.

An object of the present invention is to provide an improved method of preparing molds in which both the metal and sand parts of the mold are heated by direct firing without damaging the parts.

A more specific object is to provide a method of the foregoing type in which the parts are heated first at a relatively low temperature to avoid moisture condensation thereon and later at a relatively high temperature to condition them for receiving molten iron.

In the drawing:

FIGURE 1 is a vertical sectional view of a heating apparatus with which I can practice the method of the present invention; and

FIGURE 2 is a graph showing the relation between temperature and humidity in the apparatus.

FIGURE 1 shows a heating apparatus which includes a direct-fired chamber 10, a door 12 at the front of the chamber, a track 13 extending into the chamber through the door, burners 14 at the back of the chamber, and a flue 15. Mold parts M to be heated are placed on the truck 16 which enters and leaves the chamber along the track. A blower 17 supplies combustion air at constant volume to the burners through a duct 18 which contains a butterfly valve 19. Gaseous fuel reaches the burners through a line 20, which contains a motorized regulating valve 21. I mount a thermocouple 22 in the chamber 10 and connect the thermocouple to an automatic temperature controller 23. I connect the controller to the motor which operates the fuel-regulating valve 21. The controller has an adjustment knob 24, which I can

2

set to any temperature I wish to maintain in the chamber. The controller then automatically adjusts valve 21 to admit fuel in the proper volume to hold this temperature, as known in the art. By varying the ratio of fuel-to-air in this manner, I can maintain a flame temperature anywhere from about 300° to 2200° F. The products of combustion in the chamber are in direct contact with the mold parts M.

The mold parts M are at ambient temperature when 10 I place them in the chamber 10. I turn on the burners and set the fuel supply to maintain a flame temperature in the range of about 300° to 325° F. I set the temperature controller 23 to maintain a chamber temperature in the range of about 200° to 220° F., as registered 15 at the thermocouple 22. When the chamber is cold, the temperature controller would tend to allow a high flame temperature until the chamber reaches the temperature for which the controller is set. Hence I further limit the fuel supply at the beginning of the cycle to 20 prevent excessive flame temperature. Under these conditions the parts heat slowly and are dried. The products of combustion are at a sufficiently low concentration that moisture therein does not condense on the surface of a chill. As FIGURE 2 shows graphically, 25 the apparatus is operating in Area B below the saturation curve. Likewise there is no drastic heat applied to sand parts, such as might cause unduly rapid vaporization of the moisture therein and resultant defects. I continue to heat the mold parts under these conditions 30 for about four hours in order to bring them uniformly to a temperature of about 200° to 220° F. Thereafter I change the setting of the temperature controller 23 to maintain a chamber temperature of about 600° to 800° F. I heat the parts at the latter temperature for about eight 35 hours, after which they are uniformly at the temperature for pouring and properly dried. For convenience I can operate the controller 23 automatically by using a timer to change its setting.

From the foregoing description it is seen that my invention affords a simple effective method of preparing molds for forming cast iron rolls. The main difficulty in heating chills in a direct-fired chamber has been that moisture formed as a combustion product condenses on the chill at a start of the cycle. Such moisture causes 40 rust spots which subsequently lead to a defective casting. I overcome this difficulty by maintaining the combustion products at a low concentration until the chill is at a temperature above the dew point. The slow heating also avoids damage to the sand parts of the mold, 45 as already explained.

While I have shown and described only a single embodiment of my invention, it is apparent that modifications may arise. Therefore, I do not wish to be limited to the disclosure set forth but only by the scope of 50 the appended claims.

I claim:

1. A method of preparing mold parts for use in forming cast iron rolls comprising placing the parts at ambient temperature in a direct-fired heating chamber, 55 burning gaseous fuel in air in said chamber with the products of combustion directly contacting the parts, setting the ratio of fuel-to-air at a level which maintains a flame temperature of about 300° to 325° F. and a chamber temperature of about 200° to 220° F. for about four hours, and changing the ratio of fuel-to-air to a level 60 which maintains the chamber temperature at about 600° to 800° F. for about eight hours, whereby the parts heat slowly until they reach a temperature above the dew point and thereafter heat to a temperature for receiving molten iron.

2. A method as defined in claim 1 in which the parts include a cast iron chill and in which the slow heating

limits the products of combustion to a concentration insufficient for moisture in the products to condense on the surface of the chill until the surface reaches a temperature above the dew point.

3. A method as defined in claim 1 in which the parts 5 include sand parts initially containing 8 to 8.5 percent moisture and in which the slow heating prevents overly rapid vaporization of the moisture.

4. A method as defined in claim 1 in which the volume of air introduced to the chamber remains constant 10 and the ratio is changed by regulating the volume of fuel.

References Cited by the Examiner

UNITED STATES PATENTS

|           |         |          |       |          |
|-----------|---------|----------|-------|----------|
| 1,335,222 | 3/1920  | Davis    | ----- | 22—87    |
| 2,258,515 | 10/1941 | Mowat    | ----- | 263—52 X |
| 2,543,388 | 2/1951  | Urquhart | ----- | 263—52   |

J. SPENCER OVERHOLSER, *Primary Examiner.*

E. MAR, *Assistant Examiner.*